

[54] HEAT RESISTING  
NICKEL-ALUMINUM-MOLYBDENUM  
ALLOY

[75] Inventors: Noboru Komatsu; Takatoshi Suzuki; Nobuyuki Yamamoto; Yukikazu Tsuzuki, all of Nagoya, Japan

[73] Assignee: Kabushiki Kaisha Toyota Chuo Kenkyusho, Japan

[22] Filed: Dec. 5, 1973

[21] Appl. No.: 421,971

## [30] Foreign Application Priority Data

Dec. 14, 1972 Japan..... 47-125937

[52] U.S. Cl. .... 75/170; 75/171; 148/32; 148/32.5

[51] Int. Cl. 2..... C22C 19/03

[58] Field of Search ..... 75/170, 171; 148/32, 32.5

## [56] References Cited

## UNITED STATES PATENTS

|           |        |              |        |
|-----------|--------|--------------|--------|
| 1,461,178 | 7/1923 | Cooper ..... | 75/170 |
| 2,542,962 | 2/1951 | Kinsey ..... | 75/170 |
| 3,655,462 | 4/1972 | Maxwell..... | 75/170 |

Primary Examiner—R. Dean

Attorney, Agent, or Firm—Hill, Gross, Simpson, Van Santen, Steadman, Chiara &amp; Simpson

## [57] ABSTRACT

A nickel base heat resisting alloy having high tensile strength and excellent oxidation resistance at high temperatures in the range of 1,000°–1,200°C and toughness at room temperature characterized by the alloy comprising 91–99.9 atomic percent of a basic constituent, up to 6 atomic percent silicon, and between 0.1–3 atomic percent of a second or additive constituent consisting of one or more elements selected from a group of elements consisting of titanium, chromium, zirconium, niobium, tantalum and tungsten. The basic constituent comprises nickel, aluminum and molybdenum in the following atomic percents of the basic constituent: nickel 62–83%, aluminum 11–26%, and molybdenum 6–12%. In one embodiment, the silicon comprises 0% and the basic constituent comprises between 97–99.9 atomic percent of the alloy. In the other embodiment, the silicon is in a range of 0.5–6 atomic percent and the basic constituent is in a range of 91–99.4 atomic percent of the alloy. The addition of the silicon improves the oxidation resistance of the alloy when heated to an elevated temperature.

15 Claims, 8 Drawing Figures





Fig. 3



Fig. 1



FIG-5



FIG-2

FIG-4



FIG-6





Fig-8



## HEAT RESISTING NICKEL-ALUMINUM-MOLYBDENUM ALLOY

### BACKGROUND OF THE INVENTION

#### 1. Field of the Invention

The present invention relates to a heat resistant nickel base alloy having a high tensile strength at high temperatures and toughness at room temperature.

#### 2. Prior Art

A number of equipments and parts to be employed at high temperatures exceeding 1,000°C has increased as the result of the industrial progress and technical advancements attained during recent years. There are ever-increasing demands for heat resisting materials that can be used for parts exposed to high temperatures and heavy loads. Examples of devices which require heat resisting materials are rocket shells, atomic energy engines, combustion chambers and jet tubes or pipes for jet engines, parts of gas turbines, high temperature and high pressure apparatuses used in the chemical industries and high temperature valves. To meet the requirements for heat resisting materials, many technical studies have been conducted and, thus, many kind of heat resisting materials have been suggested. It is generally believed that heat resisting steels are applicable for use for a temperature below 800°C and that heat resisting alloys containing either nickel (Ni) or cobalt (Co) as the principle component may be used up to a temperature of 1,000°C. When used at temperatures higher than the above-mentioned temperatures, these alloys experience a deterioration in strength and therefore, their use is limited to a temperature range which does not exceed the above-mentioned temperature. In addition, the manufacture of most of these conventional alloys can involve many difficulties, for example, many of these alloys must be melted in a vacuum.

Heat resisting metal alloys, such as molybdenum (Mo), niobium (Nb) and tantalum (Ta) or ceramics may serve for a long period of time at elevated temperatures above 1,000°C. The metal alloys are inferior in their resistance to oxidation at elevated temperatures and thus are limited in their use to atmosphere or service conditions in which oxidation is not present. If they are to be used in oxidizing atmosphere, the alloy must be provided with a surface treatment for the prevention of oxidation. The ceramics have a disadvantage of a lack of ductility and thermal impact resistance. For example, ceramics will tend to break due to a sudden change in temperature. Thus, the actual use of conventional refractory or heat resisting materials at elevated temperatures posses many shortcomings and many problems with oxidation and strength at elevated temperatures still exist.

### SUMMARY OF THE INVENTION

The present invention is directed to providing a heat resisting alloy or alloys which are free from the drawbacks of the conventional heat resisting alloys as described hereinabove and which alloys have excellent mechanical strength, toughness and oxidation resistance at elevated temperatures ranging from 1,000°-1,200°C. Alloys of the present invention comprise 91-99.9 atomic percent of a basic constituent, 0.1-3 atomic percent of an additive or second constituent and up to 6 atomic percent silicon. The basic constituent comprises nickel, aluminum and molybdenum

in the following atomic percents of the basic constituent: nickel 62-83%, aluminum 11-26% and molybdenum 6-12%. The additive or second constituent consists of at least one element selected from a group of elements consisting of titanium, chromium, zirconium, niobium, tantalum and tungsten. If oxidation resistance is not a problem, the addition of the silicon can be eliminated so that the alloy contains 0 atomic percent silicon and the basic constituent will then have an atomic

5 percent of 97-99.9 atomic percent of the alloy. When the silicon is required, between 0.5-6 atomic percent is added and the basic constituent then comprises 91-99.4 atomic percent of the alloy.

### BRIEF DESCRIPTION OF THE DRAWINGS

FIG. 1 is a triangular coordinate diagram which represents by atomic percent the range of composition of the nickel, aluminum and molybdenum of the basic component or constituent of the nickel base alloy of the present invention;

FIG. 2 is a triangular coordinate diagram representing in weight percent the range of composition of the nickel, aluminum and molybdenum of the basic component or constituent of the nickel base alloy of the present invention;

FIG. 3 is a cross-sectional view of a metal melting device utilized in preparing a uni-directionally solidified rod to be used in tensile tests and other tests performed on the alloys of the present invention;

FIG. 4 is a graph illustrating the change in tensile strength at 1,000°C of different nickel-aluminum-molybdenum alloys in relationship to a variation of the content of molybdenum;

FIG. 5 is a graph illustrating the effect of changes in the molybdenum contact in a nickel-aluminum-molybdenum alloy on the measuring loads used in a toughness test at room temperature;

FIG. 6 is a graph illustrating the effect of adding different amounts of one or more additive elements of titanium, chromium, zirconium, niobium, tantalum and tungsten to a nickel-aluminum-molybdenum alloy on the tensile strength at 1,100°C;

FIG. 7 is a graph illustrating the effect of different amounts of silicon in a nickel-aluminum-molybdenum alloy of the present invention on the weight increase due to oxidation when the alloy is subjected to heating at 1,200°C for 21 hours;

FIG. 8 is a graph illustrating the changes in tensile strength at 1,100°C of the alloy of the present invention containing silicon with respect to changes in the content of silicon.

### DESCRIPTION OF THE PREFERRED EMBODIMENTS

The principles of the present invention are particularly useful for providing nickel base heat resisting alloys having a main or base constituent or component comprising nickel, aluminum and molybdenum with a second constituent or additive consisting of one or more elements selected from a group of elements consisting of titanium, chromium, zirconium, niobium, tantalum or tungsten with or without the addition of silicon which improves the resistance of the alloy to oxidation. The alloys of the present invention are a result of a study which was concentrated on improving the properties of conventional heat resisting alloys and particularly an improving of the alloys' high temperature ten-

sile strength characteristics and their toughness at room temperature. The study utilized the knowledge that an intermetallic compound of nickel and aluminum alloy, which has the formula of  $\text{Ni}_3\text{Al}$ , has an excellent resistance to oxidation at elevated temperatures when compared with conventional heat resisting alloys. The additive elements of the alloy of the present invention are for the purpose of increasing the high temperature tensile strength of the  $\text{Ni}_3\text{Al}$  alloy and the toughness at room temperatures. In addition to the additives of the second constituent, an embodiment of the alloys of the present invention includes the addition of a small quantity of silicon to increase the resistance to oxidation without detrimentally affecting the high temperature tensile strength properties.

A nickel base alloy having the following composition presents high tensile strengths at elevated temperatures as well as excellent toughness at room temperatures. The composition consists principally of nickel, aluminum and molybdenum having atomic percent of the basic component or constituent of the alloy with the percentages being enclosed by the straight lines connecting points A, B, C and D in an equilateral triangular coordinate diagram illustrated in FIG. 1. The point A in FIG. 1 represents an alloy having 83% nickel, 11% aluminum and 6% molybdenum; point B represents an alloy having 68% nickel, 26% aluminum and 6% molybdenum; point C represents an alloy having 62% nickel, 26% aluminum and 12% molybdenum; and point D represents an alloy having 77% nickel, 11% aluminum and 12% molybdenum. In addition to the basic component or constituent the alloy of the present invention includes at least an additive or second constituent which consists of at least one element selected from a group of elements consisting of titanium, chromium, zirconium, niobium, tantalum and tungsten with the basic component or constituent ranging from 97-99.9 atomic percent and the contents of the additive or second constituent ranging from 0.1-3 atomic percent. In addition, it has been found that an embodiment of the alloys of the present invention containing 91-99.4 atomic percent of the basic component or constituent, from 0.1-3 atomic percent of the additive constituent and from 0.5-6 atomic percent of silicon presents an appreciable high resistance to oxidation at elevated temperatures in addition to the high tensile strength at elevated temperatures and high toughness at room temperatures.

The triangular coordinate diagram of FIG. 1 is an equilateral triangular coordinate diagram with three sides having equal divided gradations to show the relationship between the content of nickel, aluminum and molybdenum for alloys containing more than 50 atomic percent of nickel. In the diagram of FIG. 1, the atomic percent of aluminum is plotted on the base of the triangular coordinate diagram, the atomic percent of the nickel is on the left side, and the atomic percent of the molybdenum is on the right side. Accordingly, the content of aluminum (percentages) is represented by a line extending parallel to the left side, the content of the nickel is represented by a line extending parallel to the right side and the content of molybdenum is represented by a line extending parallel to the base. For example, a point Y in FIG. 1 represents a composition consisting of 70% nickel, 10% aluminum and 20% molybdenum.

The proportions of the respective elements illustrated in FIG. 1 represent the ratio of the elements in the basic constituent; but not the ratio of the elements in an alloy which includes the additive elements. For example, if an alloy contains 98% of the basic constituent, an additive constituent of 2% titanium and the basic constituent consists of 70% nickel, 20% aluminum and 10% molybdenum, the atomic percentage of the elements of the basic constituent in the alloy are: nickel =  $70 \times 0.98 = 68.6$  atomic percent, aluminum =  $20 \times 0.98 = 19.6$  percent, molybdenum =  $10 \times 0.98 = 9.8$  percent, and titanium is 2%.

Heretofore, the amount of nickel, aluminum and molybdenum in the alloys of the present invention have been expressed in atomic percent of the basic constituent which may be between 91-99.9 atomic percent of the alloy. Using the above described calculation, the alloys of the present invention can be described in atomic percent range of the alloy as follows: nickel 56.42-82.91%; aluminum 10.01-25.974%; molybdenum 5.46-11.988%; additive constituent 0.1-3%; and silicon 0-6%. If silicon is not present, the alloys of the present invention will have the following range of atomic percents for the elements of the basic constituent: nickel 60.14-82.91% aluminum 10.67-25.974%; and molybdenum 5.82-11.988%. If silicon is present, the alloys of the present invention will have the following ranges of atomic percents for the element of the basic constituent: nickel 56.42-82.502%; aluminum 10.01-25.844%; and molybdenum 5.46-11.928%. It should be noted that if the additive constituent is 0.1% and silicon is not present or only 0.5%, the difference between the total percentage of the elements of the base constituents in the alloy and their percentage in the base constituent is extremely small.

For reference purposes, an equilateral triangular coordinate diagram which represents the ratio of nickel, aluminum, molybdenum by weight percent is shown in FIG. 2. The points A', B', C' and D' in FIG. 2 represent the same compositions as those in points A, B, C and D of FIG. 1.

The quantity of aluminum in the basic constituent of a nickel base alloy according to the present invention is restricted to a range of between 11 and 26% for the following reasons. It is well known that a nickel base heat resisting alloy, which consists of only  $\gamma$  phase at a desired high temperature, will include a solid solution of the other elements in the nickel and the alloy cannot achieve the desired strength. To achieve the increased tensile strength for the alloy at high temperature, at least a precipitate such as  $\text{Ni}_3\text{Al}$  must be dispersed in the  $\gamma$  phase or the  $\text{Ni}_3\text{Al}$  should be the principal component of the alloy. The presence of such a precipitate in a solid solution of nickel is an important factor to obtain the improved tensile strength at high temperature. Nickel-aluminum-molybdenum alloys having a composition with a range represented on the left hand side of the curve e (FIG. 1) are alloy compositions which have a low content of aluminum and are of alloy compositions in which only the  $\gamma$  phase is present at room temperature. At 1,200°C, the  $\gamma$  phase is present in all alloys which are in the area of the diagram of FIG. 1 on the left hand side of the curve f and at the 1,200°C, the tensile strength of the nickel-aluminum-molybdenum alloys having the composition within the range represented on the left hand side of the curve f is very low. In view of this information set forth above, the basic

constituent of the alloy of the present invention which constituent consists of nickel-aluminum-molybdenum has aluminum in an atomic percentage of more than 11% so that the  $\gamma$  phase and the  $\text{Ni}_3\text{Al}$  coexist at 1,200°C. In the area of the right hand side of a curve g (FIG. 1) and particularly the area where the content of the molybdenum is low, the alloys contain only a solid solution of  $\text{NiAl}$  in which nickel and molybdenum are dissolved (this solution is hereafter referred to as  $\gamma'$  phase). The nickel-aluminum-molybdenum alloy having the composition within this range has extremely low tensile strength at elevated temperatures. Likewise in the area of the diagram of FIG. 1 on the right hand side of the curve g in which area the content of molybdenum is high, the alloy when at about 1,200°C contains eutectic crystals of the  $\gamma'$  phase and the molybdenum with nickel and aluminum solidly dissolved therein and thus the alloy becomes very brittle and weak as the temperature increases. Specifically, when the  $\gamma'$  phase is suddenly cooled from the elevated temperatures, there takes place a Martensite type transformation and the alloy composed of the  $\gamma'$  phase is hardened and becomes extremely brittle. For example, the basic alloy of nickel-aluminum-molybdenum alloys of this invention contain less than 26% aluminum and provided toughness of more than 50 kg according to a toughness test method which will be described hereinafter. While a nickel-aluminum-molybdenum alloy having a composition at a point P of FIG. 1 (50% nickel, 45% aluminum, 5% molybdenum) has a low toughness of about 1 to 10 kg. Accordingly, in the basic constituent of nickel-aluminum-molybdenum of the alloy of this invention, the quantity of aluminum, is limited to less than 26% which is within the area of the left side of the curve g.

The quantity of molybdenum in the basic constituent is limited to a range of from 6-12 atomic percent as shown in FIG. 1. This is because nickel-aluminum-molybdenum alloy containing from 6-12% molybdenum have particularly high tensile strength at high temperatures and display an excellent toughness at room temperatures. When the amount of molybdenum in the basic constituent is increased and the constituent contains mainly  $\text{Ni}_3\text{Al}$ , the resulting nickel-aluminum-molybdenum alloys present peak values and high temperature tensile strength for a molybdenum content in a range of from 6-12%. Thus the quantity of molybdenum is limited to the range of 6-12 atomic percent.

In view of the reasons set forth hereinabove, the composition of the basic nickel-aluminum-molybdenum which is the basic constituent or component of the nickel base heat resisting alloy of this invention are limited to a range of from 68-83% nickel, 11-26% aluminum and 6-12% molybdenum.

The nickel base alloy of the present invention contains a second or additive constituent or component in an amount of 0.1-3 atomic percent which constituent consists of one or more elements selected from a group of elements consisting of titanium, chromium, zirconium, niobium, tantalum, tungsten. The addition of the second component or constituent provides extremely high tensile strengths at elevated temperatures. It is believed that the increase in the high tensile strength at high temperatures is based on the fact that the nickel-aluminum-molybdenum alloy is reinforced by dissolving one or more of the additive elements into the alloy as a solid solution. Namely atoms of one or more of the additive elements dissolve in the alloy are consid-

ered to be present as a solid solution in place of atoms of the elements forming the nickel-aluminum-molybdenum alloy and thereby strengthen the alloy structure. The desirable affect appears when the quantity of the additive constituent is from 0.1-3 atomic percent. The addition of less than 0.1% of the additive constituent exerts little influence on the strength of the alloy. The addition of more than 3% causes the formation of globulars or a square-flake shape crystalline structure of a large grain size in the dense structure of the nickel-aluminum-molybdenum alloy. It is considered that when a stress acts on the alloys having the large crystalline structure, the stresses will be concentrated on the large crystalline structure of the alloys and cause breakage of the alloy to occur. This is obvious from the fact that the addition of the additive elements in excess of 3% causes an abrupt decrease in the high temperature strength of the alloy. According to the results of a hardness test, it is perceived that with an increase in the quantity of the additive element or elements, the hardness gradually increases, but when the addition is more than 3%, the hardness abruptly decreases or the increase of the hardness tends to stop. The effect of the additive constituent occurs whether the additive elements of the group is added individually or in a mixture of one or more elements from the group. However, when more than one of the elements is added to the alloy, the total content of the elements should not exceed 3 atomic percent since the addition of more than 3% leads to the unfavorable phenomena described hereinabove.

In addition to the above-mentioned additive elements of the additive constituents, tests were conducted using boron as an additive element for the basic Ni-Al-Mo alloy. However, the boron did not appear to affect the high temperature tensile strength of the alloy. Therefore, the alloys of the present invention may contain a small amount of boron as an impurity.

An embodiment of the alloys of the present invention contain the basic component or constituent of nickel-aluminum-molybdenum, 0.1-3% of the additive constituent or component and from 0.5-6% of silicon and these alloys not only display high strength at elevated temperatures, toughness at room temperatures, but also have excellent oxidation resistance at elevated temperatures. The addition of the silicon greatly improves the oxidation resistance of the nickel base alloy of the present invention. The addition of between 0.5-6% silicon is greatly effective and the addition of from 2-4% silicon will provide the maximum oxidation resistance for the alloy. The addition of silicon less than 0.5% or more than 6% is improper for use in improving oxidation resistance. The addition of the silicon to the alloy causes a slight decrease in the strength of the alloy at elevated temperatures. However, the effect and the improvement in the oxidation resistance is far greater despite the decrease in strength at high temperatures.

The heat resisting alloys of the present invention will be further explained with the following test examples and embodiments showing the mechanical strength of the inventive alloy. Each of the alloys for the test samples of the following examples and embodiments was obtained from raw materials consisting of electrolytic nickel, high purity aluminum, high purity molybdenum, and high purity raw materials of the additive elements such as titanium, chromium, zirconium, niobium, tantalum and tungsten. These raw materials were sub-

jected to a high frequency melting in an alumina crucible under a protective atmosphere of argon gas and the resultant molten metal was cast into a cast product. The cast product thus attained was subjected to oxidation resistance tests, tensile tests and hardness tests which will each be described hereinbelow.

It is known that the mechanical properties of  $\text{Ni}_3\text{Al}$  greatly vary with the solidification direction, i.e.  $\text{Ni}_3\text{Al}$  has anisotropic properties. Therefore, each of the samples for the tensile tests was produced from a unidirectionally solidified rod so as to have a given direction of solidification.

To produce the test samples, a unidirectional solidification device illustrated in FIG. 3 was utilized. The device of FIG. 3 has a quartz tube 2 which has a lower end sealed with a heat resisting material 10 for retaining a sample. The quartz tube is supported and can be moved up and down by a support 8. There is provided a heat resisting glass tube 5 outside of the quartz tube 2 for the purpose of covering the inner and outer circumference of the tube 2 with an inert gas. An air tight sealing member 7 is provided on the upper end of the glass tube 5 and has a small tube 6 for introducing an inert gas into the quartz tube 2 and the glass tube 5. A high frequency induction work coil 4 surrounds the glass tube 5. Since the upper and circumferential parts of the quartz tube are covered by the sealing member 7 and the heat resisting glass 5, the inert gas introduced through the small tube 6 fills the inside of the quartz tube, and covers the outer peripheral portion of the quartz tube 2 to shut out the atmosphere. The inert is discharged to the atmosphere through the lower end of the glass tube 5.

To obtain a unidirectional solidified rod by using the above-described device, a sample 1 was placed in a bed 3 of alumina powder ( $\text{Al}_2\text{O}_3$ ) which bed is contained in the quartz tube 2. Then the air inside of the quartz tube 2 was replaced with argon gas by continuously supplying the argon gas through the small tube 6. After the argon gas has purged the air from the quartz tube, a high frequency induction current was applied to a high frequency work coil 4 to melt the sample 1 by means of heating it from the lower end or part thereof. The support 8 was gradually moved downward so that the sample 1 was solidified from the lower end thereof. In this manner a unidirectionally solidified rod for making test pieces or samples with the direction of their crystals arranged in the longitudinal direction was produced.

For the tensile tests, the test piece was made from the above stated unidirectionally solidified rod by machining the rod to a size with a length of 35 mm, a diameter in the parallel portion of 4 mm and a length in the parallel portion of 17 mm. The test piece was maintained in the test temperature ranging from 1,000°–1,100°C for 15 minutes and then tested at a tensile speed of 2.5 mm/minutes. The test results are represented in terms of tensile strength ( $\text{kg/mm}^2$ ).

For the oxidation test which examined the oxidation resisting properties of the sample, a test piece was prepared by cutting the above stated rod into a test piece having a diameter of 10 mm and a length of 10 mm. The faces of each of the test pieces was polished into a metallic surface. After weighing each of the test pieces, it was heated to 1,200°C and maintained in an air atmosphere for 21 hours. After completing the period of heating, the weight of each test sample was again

measured and the amount of oxidation would be indicated by any increase in the weight of the sample. From this test the oxidation weight ( $\Delta W_g$ ) and the spalling (flaking, exfoliation) weight ( $\Delta W_f$ ) were obtained in the following manner. Assuming that the weight of the test piece before the oxidation test is  $W_0$ , and that its surface area is  $S_0$ , that the weight of the test piece after the oxidation test is  $W_g$  and that the weight of the oxides, which spalled or flaked off, is  $W_f$ , the oxidation weight ( $\Delta W_g$ ) can be expressed as follows:

$$\Delta W_g = \frac{W_g + W_f - W_0}{S_0}$$

The spalling weight ( $\Delta W_f$ ) then can be expressed as follows:

$$\Delta W_f = \frac{W_f}{S_0}$$

These weights are expressed in  $\text{mg/cm}^2$ . Smaller values for the oxidation weight ( $\Delta W_g$ ) or the spalling weight ( $\Delta W_f$ ) indicate a better oxidation resisting property of the alloy.

For testing the toughness, test samples were pressed with a Vicker's hardness tester which is generally employed in measuring the toughness of superhard alloys. The toughness thereof was judged by the load which caused cracks around the trace of pressure or the indentation which was formed by the load during the tests. Samples that tend to produce such cracks under lighter loads were judged to be too brittle.

The samples were subjected to varied Vicker's loads of 1, 5, 10, 20, 30 and 50 kg, respectively, with each of the loads being impressed into three different areas of each sample, and each of the indentations was inspected or examined to determine whether or not cracks were produced by a given load. The maximum load (kg) that produced no cracks in all of the three impressed indentations is considered to be the degree of toughness.

#### Test Example I

FIG. 4 illustrates the relation between the tensile strength at 1,000°C for nickel-aluminum-molybdenum alloy as the percentage of molybdenum is changed from 0 to approximately 14%. The curves H, I and J of FIG. 4 correspond to lines h, i and j in the diagram of FIG. 1, respectively, and the curves H, I and J, respectively, represent the tensile strength at 1,000°C of the nickel-aluminum-molybdenum alloy having the composition represented by the lines h, i and j of FIG. 1. The percentage of the nickel-aluminum-molybdenum alloys at any desired point on the curves, H, I and J are obtained from the lines h, i and j of FIG. 1 by referring to the contents of molybdenum of the said given point, respectively. Thus, the line h, represents the composition of alloy wherein the aluminum of the  $\text{Ni}_3\text{Al}$  is replaced with molybdenum and is a line connecting  $\text{Ni}_3\text{Al}$  with the  $\text{Ni}_3\text{Mo}$  (FIG. 1). The line j represents the composition of an alloy wherein the nickel of the  $\text{Ni}_3\text{Al}$  is replaced with molybdenum while the line i is position between the lines h and j wherein molybdenum is added to the  $\text{Ni}_3\text{Al}$ .

The tensile strength curves H, I and J of FIG. 4 illustrate the maximum tensile strengths  $56 \text{ kg/mm}^2$ ,  $44$

kg/mm<sup>2</sup> and 36 kg/mm<sup>2</sup>, respectively, and the maximum strengths and obtained when the atomic percent of molybdenum is between 8-10%. The curves also illustrate that a high tensile strength is obtained over a range of 6-12% molybdenum in the nickel-aluminum-molybdenum alloy. These curves reveal that the elevated temperature tensile strength is more than 1.5 times as much as the tensile strength of 19 kg/mm<sup>2</sup> at 1,000°C of Ni<sub>3</sub>Al for the heat resisting alloy. The addition of molybdenum in excess of 12% causes an abrupt decrease of the high temperature tensile strength for the alloys. This decrease is believed to result from the fact that when molybdenum is in excess of 12%, the contents of the Ni<sub>3</sub>Mo in the alloy exceeds the content of the Ni<sub>3</sub>Al in the alloy. On the other hand when the content of molybdenum is less than 5%, the degree of strengthening the solid solution of Ni<sub>3</sub>Al due to molybdenum is considerably low.

#### Test Example II

FIG. 5 illustrates a relationship between the toughness at room temperature for the nickel-aluminum-molybdenum alloy and a varying percentage content of molybdenum. The illustrated alloys include a range of the basic constituent of the nickel based alloy of the present invention. The test samples were selected from a nickel-aluminum-molybdenum alloy having a composition represented by the line *h* in FIG. 1 and the contents of the nickel and the aluminum in each test sample are obtained from the line *h* of FIG. 1 by referring to the percentage content of the molybdenum of each test sample. The toughness of each of the test samples is illustrated from the data of FIG. 5.

As will be apparent from the curve of FIG. 5, in the case of more than 10% molybdenum, the toughness exceeds the critical load of 50 kg for the toughness test and the degree of toughness is too high to measure by this measuring method. This reveals that the alloys consisting of the elements nickel-aluminum-molybdenum which alloys are within the range of the basic constituent of the nickel base alloy of the present invention, namely those alloys with more than 10% molybdenum in content have a high toughness of more than 50 kg which is 2.5 times as much as the toughness of 20 kg of the conventional alloy consisting of Ni<sub>3</sub>Al without molybdenum. Thus, the alloys of the present invention have overcome the problem of insufficient toughness which was experienced in the conventional heat resisting alloys and thus are alloys with a good ductility.

#### Test Example III

In FIG. 6, the results of tensile tests at 1,100°C of an alloy containing a basic constituent of nickel-aluminum-molybdenum with the 75% nickel, 15% aluminum and 10% molybdenum and an additive constituent consisting of one or more elements of titanium, chromium, zirconium, niobium, tantalum and tungsten being added to the alloy are illustrated with the percentage of the additive constituent being from 0-5 atomic percent. The ordinate represents the tensile strength (kg/mm<sup>2</sup>) and the abscissa represents the content of the additive element or constituent. In FIG. 6, the curve *R* represents the maximum tensile strength for respective contents of the additive element and the curve *T* represents the minimum tensile strength. FIG. 6 shows that the alloys obtained by the addition of the additive element or constituent to the basic constituent of nickel-aluminum-molybdenum provides a tensile strength ranging from between the curves *R* and *T*. As

seen in FIG. 6, the minimum addition of the additive constituent causes an abrupt increase in the tensile strength to obtain the maximum value in the content ranging from 0.5-2.5% and the maximum tensile strength is 54 kg/mm<sup>2</sup> and the lower limit of the strength is 43 kg/mm<sup>2</sup>. Compared with the tensile strength of 38 kg/mm<sup>2</sup> of the nickel-aluminum-molybdenum alloy without containing the additive element, the tensile strength of the nickel-aluminum-molybdenum alloy containing the additive constituent has an increase of 15 to 40%. Additions of the additive constituent in excess of 3% however causes an abrupt decrease in the tensile strength.

#### Test Example IV

Results of oxidation resistance tests are illustrated in FIG. 7. The alloy to be tested consisted of a nickel-aluminum-molybdenum basic constituent consisting of 75% nickel, 15% aluminum and 10% molybdenum and an additive constituent of 0.6% niobium. Added to this element was 0-12% silicon and the alloys were heated at 1,200°C in an air atmosphere for 21 hours. The weight increase due to oxidation (mg/cm<sup>2</sup>) is represented on the ordinate and the content of silicon is represented on the abscissa. The results of the oxidation tests as shown in FIG. 7, are such that the addition of 0.7% silicon reduced the weight increase due to oxidation from 23.5 mg/cm<sup>2</sup> for the alloy consisting of the basic components plus the niobium as an additive constituent without silicon to 1.7 mg/cm<sup>2</sup>. This means that the addition of silicon imparts the oxidation resisting property to the alloy. Particularly, the addition of 1-4% silicon minimizes the weight increase due to oxidation to less than 2 mg/cm<sup>2</sup> and thus provides an alloy with a greatly improved oxidation resistance. However, the addition of silicon in excess of 4% causes an increase in the weight increase due to oxidation and in excess of 6% lowers the effect of improving the oxidation resistance. It was confirmed that the effect of enhancing the oxidation resistance by addition of silicon as illustrated by FIG. 7 also occurs when silicon is added to the alloys of the present invention which contain an additive agent such as titanium, chromium, zirconium, tantalum and tungsten.

The spalling weight was measured simultaneous with the measurement of the weight increased due to oxidation and presents four times as much as the weight increase due to oxidation. The addition of silicon also reduces the spalling weight in a manner similar to the decrease of the oxidation weight. This proves that the oxidation in the nickel-aluminum-molybdenum alloy proceeds with spalling. According to other tests, the addition of silicon to the nickel-aluminum alloy which contains no molybdenum did not produce any improvement in oxidation resistance.

#### Test Example V

Results of a tensile test at 1,100°C of alloys which consist of nickel-aluminum-molybdenum alloy with a basic constituent containing 75% nickel, 15% aluminum, 10% molybdenum, an additive constituent of 0.3% tantalum and various amounts of silicon in a range of 0-6% are illustrated in FIG. 8. The tensile strength (kg/mm<sup>2</sup>) is represented by the ordinate and the content of silicon is represented by the abscissa. As seen in FIG. 8, the tensile strength follows substantially a linear decrease with an increase in the content of silicon and the tensile strength of the nickel-aluminum-molybdenum alloy without containing silicon is approx-

imately 50 kg/mm<sup>2</sup>. The nickel-aluminum-molybdenum alloy containing 6% silicon has a tensile strength lower to approximately 30 kg/mm<sup>2</sup>. The decrease in the tensile strength at high temperatures due to the addition of silicon is commonly found in all of the nickel-aluminum-molybdenum alloys containing one or more of the additive elements and silicon. In view of the decrease of the tensile strengths at high temperatures, the addition of excessive silicon is not desirable. Since the conventional Ni<sub>3</sub>Al alloy has a tensile strength of less than 19 kg/mm<sup>2</sup> at 1,000°C and less than 10 kg/mm<sup>2</sup> at 1,100°C, it is concluded that the alloys having a tensile strength of 30 kg/mm<sup>2</sup> at 1,100°C is excellent particularly if it has a heat resisting strength or property.

#### Embodiment I

Twenty-four samples of the alloys according to the present invention were prepared from electrolytic nickel, high purity aluminum, high purity molybdenum and high purity titanium, chromium, zirconium, niobium, tantalum and tungsten were prepared by melting in the argon gas atmosphere. These samples which have an atomic percent composition set forth in Table I were subjected to test for tensile strength at 1,100°C, for oxidation resistance at 1,200°C for 21 hours and toughness test at room temperature. The results of the tests for each sample are given in the Table I. The alloy numbers 1 through 17 have a composition close to the point K within the range of the basic constituents shown in FIG. 1. The alloys 18 through 20 and the alloys 21 through 24 have, respectively, compositions close to the points L and M which are both within the range of the basic constituents shown in FIG. 1.

For reference, the following Table I gives the results of the same tensile tests, oxidation resistance test for the alloys having a composition equal to those taken at points K, L, M of FIG. 1 and for Inconel 713C, which is a conventionally known heat resisting alloy.

30

35

As will be apparent from Table I, the alloys of this invention contain the basic constituent of nickel-aluminum-molybdenum and at least one element of titanium, chromium, zirconium, niobium, tantalum and tungsten present extremely high tensile strengths at elevated temperatures. For example, the tensile strength of alloys 1 through 17 consisting of the alloy K which has a composition of point K in FIG. 1 and additive element such as titanium is from 43 to 54 kg/mm<sup>2</sup> approximately and this is higher by 5 to 16 kg/mm<sup>2</sup> than the elevated temperature strength of 38 kg/mm<sup>2</sup> of the alloy K without any of the additive elements. Alloys of the present invention having a base constituent comprising the alloys L or M and one or more additive elements hereinbefore described have a tensile strength at high temperatures from approximately 35 to 39 kg/mm<sup>2</sup>, and from about 30 to 32 kg/mm<sup>2</sup>, respectively. These alloys are higher in tensile strength by 5 to 9 kg/mm<sup>2</sup> and by 5 to 7 kg/mm<sup>2</sup> in comparison with the tensile strength of 30 kg/mm<sup>2</sup> and the tensile strength of 25 kg/mm<sup>2</sup> of the basic alloys L and M, respectively. None of the alloys presented have a toughness of less than 50 kg. This means that the alloys of the present invention have excellent toughness properties at room temperature. In view of the fact that the tensile strength at high temperature for Inconel 713C (the conventionally known excellent heat resisting alloy) is 14.0 kg/mm<sup>2</sup>, it can be concluded that the tensile strengths at high temperatures ranging from 30 to 54 kg/mm<sup>2</sup> for the alloys of the present invention are extremely good.

#### Embodiment II

Some of the same alloys as those used in the table of Embodiment I, and a high purity silicon were melted under an argon gas atmosphere to prepare six kinds of alloys having a composition shown in Table II. Alloys number 30 through 35 are equivalent to the alloys number 1, 3, 5, 7, 10 and 13 which are tabulated in Table I and have approximately 2% silicon added

TABLE I

| Alloy No.    | Composition (Atomic percent). |       |      |                     |      |                    |      |                    | Tensile test at 1100°C |                                | Weight increase due to oxidation (mg/cm <sup>2</sup> ) | Toughness (kg) |              |
|--------------|-------------------------------|-------|------|---------------------|------|--------------------|------|--------------------|------------------------|--------------------------------|--------------------------------------------------------|----------------|--------------|
|              | Ni                            | Al    | Mo   | Ti                  | Cr   | Zr                 | Nb   | Ta                 | W                      | Strength (kg/mm <sup>2</sup> ) | Elongation (%)                                         |                |              |
| 1            | 74.16                         | 14.79 | 9.85 | 1.20                | —    | —                  | —    | —                  | —                      | 49.9                           | 8                                                      | 28.7           | more than 50 |
| 2            | 73.26                         | 14.61 | 9.73 | 2.40                | —    | —                  | —    | —                  | —                      | 53.6                           | 8                                                      | 33.0           | "            |
| 3            | 74.23                         | 14.80 | 9.86 | —                   | 1.11 | —                  | —    | —                  | —                      | 43.8                           | 10                                                     | 4.8            | "            |
| 4            | 73.42                         | 14.63 | 9.76 | —                   | 2.19 | —                  | —    | —                  | —                      | 43.8                           | 10                                                     | 3.5            | "            |
| 5            | 74.58                         | 14.87 | 9.91 | —                   | —    | 0.64               | —    | —                  | —                      | 44.0                           | 6                                                      | 28.3           | "            |
| 6            | 74.12                         | 14.77 | 9.85 | —                   | —    | 1.26               | —    | —                  | —                      | 42.9                           | 7                                                      | 36.3           | "            |
| 7            | 74.59                         | 14.87 | 9.91 | —                   | —    | —                  | 0.63 | —                  | —                      | 48.0                           | 9                                                      | 23.5           | "            |
| 8            | 74.12                         | 14.78 | 9.85 | —                   | —    | —                  | 1.25 | —                  | —                      | 49.1                           | 9                                                      | 29.0           | "            |
| 9            | 73.16                         | 14.59 | 9.72 | —                   | —    | —                  | 2.53 | —                  | —                      | 44.7                           | 7                                                      | 34.0           | "            |
| 10           | 74.82                         | 14.92 | 9.94 | —                   | —    | —                  | —    | 0.32               | —                      | 49.1                           | 9                                                      | 5.3            | "            |
| 11           | 74.56                         | 14.88 | 9.91 | —                   | —    | —                  | —    | 0.65               | —                      | 50.7                           | 11                                                     | 7.8            | "            |
| 12           | 74.06                         | 14.77 | 9.85 | —                   | —    | —                  | —    | 1.32               | —                      | 52.3                           | 8                                                      | 10.8           | "            |
| 13           | 74.83                         | 14.92 | 9.94 | —                   | —    | —                  | —    | —                  | 0.31                   | 48.7                           | 8                                                      | 21.9           | "            |
| 14           | 74.58                         | 14.87 | 9.91 | —                   | —    | —                  | —    | —                  | 0.64                   | 52.7                           | 11                                                     | 26.1           | "            |
| 15           | 74.31                         | 14.83 | 9.88 | —                   | —    | —                  | 0.65 | —                  | 0.33                   | 53.6                           | 10                                                     | 49.5           | "            |
| 16           | 73.50                         | 14.70 | 9.80 | —                   | 1.00 | —                  | —    | 1.00               | —                      | 53.0                           | 7                                                      | 5.0            | "            |
| 17           | 73.35                         | 14.67 | 9.78 | 1.00                | —    | 1.20               | —    | —                  | —                      | 51.2                           | 6                                                      | 48.4           | "            |
| 18           | 69.16                         | 19.76 | 9.88 | 1.20                | —    | —                  | —    | —                  | —                      | 38.1                           | 11                                                     | 15.4           | "            |
| 19           | 69.07                         | 19.74 | 9.87 | —                   | —    | —                  | —    | 1.32               | —                      | 39.0                           | 9                                                      | 8.7            | "            |
| 20           | 69.30                         | 19.80 | 9.90 | —                   | —    | —                  | 1.00 | —                  | —                      | 35.0                           | 12                                                     | 13.4           | "            |
| 21           | 66.79                         | 22.93 | 9.97 | —                   | —    | —                  | —    | —                  | 0.31                   | 36.0                           | 26                                                     | 3.0            | "            |
| 22           | 66.56                         | 22.85 | 9.94 | —                   | —    | 0.65               | —    | —                  | —                      | 30.4                           | 14                                                     | 5.4            | "            |
| 23           | 66.00                         | 22.65 | 9.85 | 1.50                | —    | —                  | —    | —                  | —                      | 32.2                           | 20                                                     | 4.7            | "            |
| 24           | 66.56                         | 22.85 | 9.94 | —                   | —    | —                  | —    | 0.65               | —                      | 32.1                           | 19                                                     | 2.6            | "            |
| K            | 75                            | 15    | 10   | —                   | —    | —                  | —    | —                  | —                      | 38.0                           | 2                                                      | 39.3           | "            |
| L            | 70                            | 20    | 10   | —                   | —    | —                  | —    | —                  | —                      | 30.0                           | 12                                                     | 7.0            | "            |
| M            | 67                            | 23    | 10   | —                   | —    | —                  | —    | —                  | —                      | 25.1                           | 21                                                     | 2.0            | "            |
| Inconel 713C | 74.2                          | 6.1   | 4.2  | B: 0.012<br>Zr: 0.1 |      | Ti: 0.8<br>Nb: 2.0 |      | Cr: 12.5<br>C: 0.1 | 14.0                   | —                              | 2.5                                                    | —              |              |

thereto. These alloys numbers 30 through 35 were each tested for tensile strength of 1,100°C, oxidation resistance at 1,200°C for 21 hours and toughness property at room temperature by the same methods that were utilized for the alloys of Embodiment I. The results of these tests are given in the following Table II.

TABLE II

| Alloy No. | Composition (Atomic percent) |       |      |      |      |      |      |      | Tensile test at 1100°C |      | Weight increase due to oxidation (mg/cm <sup>2</sup> ) | Toughness (kg) |     |         |
|-----------|------------------------------|-------|------|------|------|------|------|------|------------------------|------|--------------------------------------------------------|----------------|-----|---------|
|           | Ni                           | Al    | Mo   | Ti   | Cr   | Zr   | Nb   | Ta   | W                      | Si   | Strength (kg/mm <sup>2</sup> )                         | Elongation (%) |     |         |
| 30        | 72.67                        | 14.48 | 9.66 | 1.18 | —    | —    | —    | —    | —                      | 2.01 | 39.3                                                   | 3.9            | 2.4 | more    |
| 31        | 72.74                        | 14.50 | 9.67 | —    | 1.08 | —    | —    | —    | —                      | 2.01 | 36.2                                                   | 7.0            | 1.7 | than 50 |
| 32        | 73.05                        | 14.56 | 9.71 | —    | —    | 0.62 | —    | —    | —                      | 2.06 | 37.1                                                   | 4.0            | 5.2 | "       |
| 33        | 73.06                        | 14.56 | 9.71 | —    | —    | —    | 0.61 | —    | —                      | 2.06 | 43.9                                                   | 5.0            | 1.7 | "       |
| 34        | 73.32                        | 14.60 | 9.74 | —    | —    | —    | —    | 0.31 | —                      | 2.03 | 44.3                                                   | 3.8            | 1.2 | "       |
| 35        | 73.33                        | 14.71 | 9.74 | —    | —    | —    | —    | —    | 0.31                   | 2.03 | 45.4                                                   | 7.0            | 1.7 | "       |

When a comparison of the alloys 30 through 35 of 20 the present embodiment is made with the alloys numbers 1, 3, 5, 7 10 and 13 which do not contain silicon as shown in the tabulation of Table I, the alloys of this embodiment exhibit from one-third to one-fifth of the amount of weight increase due to oxidation as their 25 corresponding alloys which contained no silicon. This means that the oxidation resistance of these alloys of this embodiment was greatly improved by the addition of silicon. The tensile strengths of the alloys of this embodiment however, are somewhat lower by approximately 10-20% due to the addition of silicon. In view of the fact that the tensile strength of the alloys of this embodiment at 1,100°C range from 36 to 45 kg/mm<sup>2</sup> and the weight increase due to oxidation after heating 30 at 1,200°C for 21 hours is from 1.2-5.2 mg/cm<sup>2</sup>, it is believed that the alloys of this embodiment are excellent in high temperature strength and in oxidation resistance. It is apparent from a comparison of test results 35 of Table II with the test results for Inconel 713C in Table I in which the Inconel 713C has a tensile strength of 14.2 kg/mm<sup>2</sup> at 1,100°C and a weight increase due to oxidation of 2.5 mg/cm<sup>2</sup> when heated to 1,000°C for 21 hours. In addition the test results of the alloy numbers 30 through 35 show that at room temperature, the results of the toughness test was more than 50 kg. This clearly teaches that these alloys have excellent toughness particularly at room temperature.

In summary, the heat resisting alloys of the present invention which consists of three basic elements such as nickel, aluminum and molybdenum as a basic constituent whose composition falls in a range defined by the points, A, B, C and D in FIG. 1 and includes 0.1-3 atomic percent of one or more elements of titanium, chromium, zirconium, niobium, tantalum and tungsten exhibit greatly improved tensile strengths at elevated temperatures and excellent toughness at room temperature. The alloys consisting of the basic constituents comprising nickel-aluminum-molybdenum having the above-mentioned composition, one or more additive elements mentioned above and from 0.5-6 atomic percent silicon exhibit high tensile strengths at elevated temperatures, excellent toughness properties at room temperature and also having excellent oxidation resistance properties at elevated temperatures. Thus, the alloys of the present invention are versatile as heat resisting materials which are applicable for use in steam turbines, gas turbines, devices for use in chemical in-

dustry or device which require operation at elevated temperatures.

Although minor modifications might be suggested by those versed in the art, it should be understood that we wish to employ within the scope of the patent granted hereon all such modifications as reasonably and prop-

erly come within the scope of our contribution to the art.

We claim:

1. A heat resisting alloy which has excellent mechanical strength, toughness and oxidation resistance at elevated temperatures in the range of 1,000°-1,200°C, said alloy consisting essentially of 93-98.9 atomic percent of a basic constituent comprising nickel, aluminum and molybdenum in the following atomic percents of the basic constituent, nickel 62-83%, aluminum 11-26%, and molybdenum 6-12%; 0.1-3 atomic percent of a second constituent consisting of at least one element selected from a group consisting of titanium, chromium, zirconium, niobium, tantalum and tungsten; and 1-4 atomic percent silicon.

2. A heat resisting alloy according to claim 1, wherein the silicon is present in a range of 2-4 atomic percent.

3. A heat resisting alloy according to claim 1, 40 wherein the second constituent is present in a range of 0.5-2.5 atomic percent.

4. A heat resistance alloy which has excellent mechanical strength, toughness and oxidation resistance at elevated temperatures in a range of 1,000°-1,200°C, 45 said alloy consisting essentially of the following atomic percentages of constituents:

56.42 - 82.502% nickel;

10.01 - 25.844% aluminum;

5.46 - 11.928% molybdenum;

1 - 4% silicon; and

0.1 - 3% of an additive constituent, selected from a group of elements consisting of titanium, chromium, zirconium, niobium, tantalum, and tungsten, said additive constituents comprising at least one of said elements from said group.

5. A heat resisting alloy according to claim 4, 60 wherein the additive constituent is titanium in the range of 1-2.4 atomic percent.

6. A heat resisting alloy according to claim 4 wherein the additive constituent is chromium in a range of 1.0-2.5 atomic percent.

7. A heat resisting alloy according to claim 4, 65 wherein the additive constituent comprises zirconium in a range of 0.5-1.5 atomic percent.

8. A heat resisting alloy according to claim 4, 70 wherein the additive constituent comprises niobium in a range of 0.5-2.6 atomic percent.

9. A heat resisting alloy according to claim 4, wherein the additive constituent comprises tantalum in a range of 0.32-1.32 atomic percent.

10. A heat resisting alloy according to claim 4, wherein the additive constituent comprises tungsten in a range of 0.31-0.64 atomic percent.

11. A heat resisting alloy according to claim 4, wherein the additive constituent comprises both niobium and tungsten.

12. A heat resisting alloy according to claim 4, wherein the additive constituent comprises both chromium and tantalum.

13. A heat resisting alloy according to claim 4, wherein the additive constituent comprises both titanium and zirconium.

14. A heat resisting alloy according to claim 4, wherein the silicon is in a range of 2.0-2.1%; the nickel is in a range of 72.67-73.33%; the aluminum is in a range of 14.48-14.71%; the molybdenum is in a range of 9.66-9.74%; and the additive constituent is in a range of 0.31-1.18%.

15. A heat resisting alloy according to claim 4, wherein the silicon is in a range of 2-4%.

\* \* \* \* \*

15

20

25

30

35

40

45

50

55

60

65